# EUROPEAN PATENT SPECIFICATION

(11) **EP 3 918 955 B1**
(45) Date of publication and mention of the grant of the patent: **01.04.2026**
(21) Application number: 20188616.5
(22) Date of filing: 30.07.2020
(51) Int. Cl.: A47C 27/22, A47C 7/20

(54) **COMPOSITE FILLING FOR A SEAT**
KOMPOSITFÜLLUNG FÜR EINEN SITZ
REMPLISSAGE COMPOSITE POUR UN SIÈGE

(30) Priority: 05.06.2020 CZ 202037619 U
(43) Date of publication of application: 08.12.2021
(73) Proprietor: Technicka univerzita v Liberci, 460 01 Liberec (CZ)
(72) Inventor: Fliegel, Vitezslav, 460 15 Liberec (CZ); Martonka, Rudolf, 460 01 Liberec (CZ); Srb, Pavel, 460 05 Liberec (CZ); Lepsik, Petr, 466 04 Jablonec nad Nisou (CZ)
(74) Representative: Musil, Dobroslav

(56) References cited:
- JP-A- H05 269 031
- US-A1- 2011 169 320
- US-A1- 2019 023 861

## Description

### Technical field

The invention relates to a composite filling for a seat comprising polyurethane foam, wherein the filling is divided in the direction of its height into at least three regions, at least two the load regions comprising polyurethane foam with fibers which are firmly connected to the polyurethane foam.

### Background art

Polyurethane foam, which is easily shaped and deformable, is used to fill the bottom seat and backrests of seats, especially car seats, mattresses and sofas. When polyurethane foam is loaded, e.g. when a person sits on the bottom seat, the polyurethane foam is compressed and deformed, thus providing a certain static and dynamic comfort for the seated person.

The disadvantage of the seats the filling of which is made of a filling composed of polyurethane foam, is its large deformation, when at a certain level of load the maximum compression of the polyurethane foam occurs, which results in the polyurethane foam losing its comfort properties. This disadvantage is solved by increasing the thickness or density of the polyurethane foam, which, however, increases the height of the seat and increases the production costs.

JPH05269031A describes a filling comprising, see paragraph [0009], a surface leather, a non-woven fabric attached to the back of the surface leather and a polyurethane foam attached to the back of the non-woven fabric. The nonwoven fabric has a two-layer structure comprising a higher density upper layer and a lower density lower layer, wherein the lower density lower layer is impregnated with the polyurethane foam of the polyurethane foam layer to form a fiber reinforced polyurethane layer. As described in paragraph [0012], the underside of the polyurethane foam can be reinforced in a similar manner, i.e., by impregnating the underside of the polyurethane foam to form a fiber-reinforced polyurethane foam. The polyurethane foam with fibers is described in more detail in paragraph [0014], wherein, "to increase the hardness of the filling, a thick fiber-reinforced polyurethane layer can be formed by molding the nonwoven fabric ". In Fig.5 and Fig 6, the polyurethane layer is reinforced with a flat non-woven fabric, not individual fibers. The arrangement of the individual layers is such that the density of the individual layers increases and decreases irregularly and in leaps and bounds, with only some of the layers containing polyurethane foam, only some of the layers containing nonwoven fabric, and none of the layers containing individual fibers.

US2019/023861A1 in par. [0010] describes a filling that includes a packaging material comprising a foam material suspended from a fiber net. The packing material is necessary to secure the fiber net [0019] and to prevent the foam material from falling out of the inner portion of the filling. This inner part of the filling is formed by foam particles, par. [0024], [0032] and Fig. 1 to Fig. 4, which are suspended on the fibers and placed loosely between the fibers of the fiber net [0019]. The foam particles are separated from each other by the fiber mesh to create air gaps between the foam particles [0032].

US2011/0169320A1 describes a filling containing fibers, foam particles and a bonding material [0005]. The prior art as described in this document describes that the latex, paragraph [0008], [0019] or [0021], which together with the fibers forms the main load-bearing part of the filling, is the bonding material of the claimed solution. In order to increase seating comfort, foam particles are added to the top of the filling which do not touch each other and are therefore separated from each other by [0021] latex. The foam particles are preferably formed by the latex itself [0019] in the shape of hollow spheres [0020]. The filling is formed by fiber-reinforced latex, with foam particles added to the top of the filling to increase comfort. The object of the present invention is providing a filling for a seat comprising polyurethane foam which has an increased load-bearing capacity, while maintaining the same height and density, or which has the same load-bearing capacity with reduced height or density of the polyurethane foam.

### Principle of the invention

The object of the invention is achieved by a filling for a seat whose principle consists of the fact that the uppermost region contains the polyurethane foam substantially free of fibers, with other immediately adjacent load regions arranged below it, having a downwardly increasing density of fibers in the polyurethane foam.

In a preferred embodiment, the filling for a seat comprises four superimposed regions, wherein the uppermost region has a zero fiber density, and the second light load region arranged below it has a fiber density in the polyurethane foam of from 1 to 10 kg/m³, the third middle load region arranged below has a fiber density in the polyurethane foam of 10 to 15 kg/m³ and the fourth heavy load region arranged below has a fiber density in the polyurethane foam of 15 to 20 kg/m³.

The fibers are arranged in the polyurethane foam in the horizontal direction or in the vertical direction, or they are arranged chaotically or the fibers are arranged in different directions in the individual regions of the polyurethane foam.

### Description of the drawings

Exemplary embodiments of the seat filling according to the invention are shown in the accompanying drawings, where the polyurethane foam in Fig. 1 comprises fibers arranged in the horizontal direction, in Fig. 2 it comprises fibers arranged in the vertical direction and in Fig. 3 it comprises fibers arranged chaotically.

### Examples of embodiment

The seat filling according to the invention comprises polyurethane foam **1,** which is saturated with fibers **2** in such a manner that the individual fibers 2 are firmly connected to the polyurethane foam and thus form a composite material. The bulk density of the fibers in the polyurethane foam **1** ranges from 1 to 40 % of the total bulk density of the filling, whereby at a higher bulk density of the fibers in the polyurethane foam **1** the polyurethane foam **1** acquires a higher load-bearing capacity and thus deforms less under load. To ensure that the polyurethane foam **1** in the seat filling retains its load-bearing properties, the bulk density of the polyurethane foam **1** must be at least 60 % of the total bulk density of the filling.

The filling for a seat consists of at least two load regions **4, 5, 6,** which comprise composite polyurethane foam **1** saturated with fibers **2**, whereby se the individual load regions differ in the density of the fibers **2** in the polyurethane foam **1.** In the variant of embodiment shown, there is no firm division between these load regions, since they merge into one another. Hereinafter, a particularly advantageous variant of embodiment will be disclosed, which comprises three load regions **4**, **5**, **6**, namely a region **4** of light load and/or a region **5** of middle load and/or a region **6** of heavy load. These regions differ in the density of the fibers **2** in the composite polyurethane foam **1,** which is particularly suitable for loading by a seated person. The composite polyurethane foam **1** comprises at least two load regions **4, 5**, **6,** they are arranged one above the other so that the region with lower density of the fibers **2** in the polyurethane foam **1** is placed above the region with higher density of the fibers **2.** As the composite polyurethane foam **1** is compressed, the load regions **4, 5**, **6** are gradually compressed from top to bottom. Since there is a higher density of the fibers **2** in each further lower load region **4**, **5**, **6**, each further load region **4**, **5, 6** has a higher load capacity and less compression, thus achieving adjustable stiffness over the whole height and a wide range of possible loads without losing seating comfort. Depending on the desired properties of the final product, the fibers in the individual load regions **4**, **5**, **6** are arranged either in the horizontal or vertical direction or chaotically in different directions. To increase the comfort of the seated person, there is a comfort region **3** in the upper part of the filling, which is formed by polyurethane foam **1** which does not contain any fibers **2.**

In one variant of embodiment, synthetic fibers, such as polyamide fibers, polyester fibers, silon fibers, etc., are used as fibers **2**, while in another variant of embodiment, natural fibers are used, such as flax, coconut, African grass, cotton, etc.

In the exemplary embodiments shown in Fig. 1, Fig. 2 and Fig. 3, the polyurethane foam **1** of the seat comprises in total four regions with a different density of the fibers **2** in the polyurethane foam **1,** whereby in Fig. 1 the fibers **2** in the polyurethane foam **1** are arranged in the horizontal direction, in Fig. 2 the fibers **2** in the polyurethane foam **1** are arranged in the vertical direction and in Fig. 3 the fibers **2** in the polyurethane foam **1** are arranged chaotically.

The first comfort region **3** is located at the top of the polyurethane foam **1,** i.e. the side which will face upwards when the seat is positioned in its place, and there are essentially no fibers **2** arranged in it. This region serves as a comfort region for increased comfort and as a thermo area to maintain the temperature on the surface of the first comfort region **3.** Under the first comfort region **3** is arranged a second region **4** of light load in which arranged in the polyurethane foam **1** are fibers **2** whose density in the polyurethane foam **1** is greater than in the first comfort region **3.** Under the second region **4** of light load is arranged a third region **5** of middle load, in which in the polyurethane foam **1** are arranged fibers **2** whose fiber **2** density in the polyurethane foam **1** is greater than the density of the fibers **2** in the polyurethane foam **1** in the second region **4** of light load. Under the third region **5** of middle load is arranged a fourth region **6** of heavy load, in which in the polyurethane foam **1** are arranged fibers **2,** whereby the density of the fibers **2** in the polyurethane foam **1** in the fourth region **6** of heavy load is greater than the density of the fibers **2** in the polyurethane foam **1** in the third region **5** of middle load.

In the standard embodiment, the height of the first comfort region **3** is in the range of 10 to 15 mm and only serves to increase the comfort of the seated person and for air conditioning. The heights of the light, medium and heavy load regions **4**, **5**, **6** are identical in the embodiment shown, i.e. they evenly distribute the remaining height of the polyurethane foam **1** without the first comfort region **3.** In another embodiment, the height of the individual load regions **4**, **5**, **6** is unevenly distributed.

Each region **3, 4**, **5**, **6** of the polyurethane foam **1** has a different load-bearing capacity depending on the density of the fibers **2** arranged in it. By changing the number of fibers **2** in individual regions **3, 4**, **5**, **6**, i.e., by changing the density of the fibers **2** in the polyurethane foam **1,** the total load-bearing capacity of the resulting seat filling changes.

Another factor which partly influences the overall load-bearing capacity of the seat filling is the direction in which the fibers are arranged **2** in the polyurethane foam **1.** In a variant shown in Fig. 1 the fibers **2** in the polyurethane foam **1** are arranged in the horizontal direction in which the filling has the most compact dimensions, but the least load-bearing capacity. In a variant shown in Fig. 2, the fibers **2** in the polyurethane foam **1** are arranged in the vertical direction, in which the filling has a greater load-bearing capacity at the same fiber **2** density **2,** but also larger dimensions. In the variant shown in Fig. 3, the fibers **2** in the polyurethane foam **1** are arranged chaotically, i.e. the fibers **2** directed randomly in all directions, in which the filling has omnidirectional strength and is the simplest to manufacture. In another embodiment not shown, the fibers **2** are arranged in at least two load regions **4**, **5**, **6** in different directions, i.e. horizontally in one of the load regions **4, 5, 6** and vertically in the remaining load regions **4, 5, 6.**

To reduce the production costs of the seat filling, the production density of the polyurethane foam **1,** which is costly, is reduced and the lost load-bearing capacity of the filling is replaced by adding a number of fibers **2** of different densities in at least two load regions **4**, **5**, **6** of the polyurethane foam **1.**

In an exemplary embodiment, the composite polyurethane foam **1** comprises in total four regions **3, 4, 5, 6** with a different density of the fibers **2.** In the first comfort region **3,** there is zero density of the fibers **2,** i.e., no fibers **2** are arranged in this comfort region **3.** In the second region **4** of light load, the density of the fibers **2** in the polyurethane foam **1** is in the range of 1 to 10 kg/m³. In the third region **5** of middle load, the density of the fibers **2** in the polyurethane foam **1** is in the range of 10 to 15 kg/m³. In the fourth region **6** of heavy load, the density of the fibers **2** in the polyurethane foam **1** is in the range of 15 to 20 kg/m³.

In another embodiment, the number of at least two load regions **4**, **5**, **6** in the polyurethane foam **1** varies depending on the desired properties of the resulting filling and the bulk density of the fibers **2** in the polyurethane foam **1** is adapted in a manner known to the person skilled in the art in the range of 1 to 40 % of the volume of the polyurethane foam **1.** To reduce the cost of producing the seat filling while maintaining its sufficient load-bearing capacity, the density of the polyurethane foam **1** is reduced by 1 to 10 %, i.e. to 90 to 99 % of the original density of the polyurethane foam **1.**

## Claims

1. A filling for a seat comprising polyurethane foam (1), the filing consisting of at least two load regions (4, 5, 6), which comprise composite polyurethane foam (1) saturated with fibers (2) which are firmly connected to the polyurethane foam (1), wherein the individual load regions (4, 5, 6) differ in the density of the fibers (2) in polyurethane foam (1), wherein the load regions (4, 5, 6) are arranged one above another so that the load region with lower density of the fibers (2) in the polyurethane foam (1) is placed above the load region with higher density of the fibers (2) in the polyurethane foam (1) and wherein in the upper part of the filing, there is a comfort region (3) formed by polyurethane foam (1), which does not contain any fibers (2)..

2. A filling according to claim 1, **characterized in that,** it consists of four regions (3, 4, 5, 6), wherein in first comfort region (3), there is zero density of the fibers (2), in the second region (4) of light load, the density of the fibers in the polyurethane foam (1) is in the range of 1 to 10 kg/m³, in the third region (5) of middle load, the density of the fibers (2) in the polyurethane foam (1) is in the range of 10 to 15 kg/m³ and in the fourth region (6) of heavy load, the density of the fibers (2) in the polyurethane foam (1) is in the range of 15 to 20 kg/m³.

3. The filling for a seat according to any of the preceding claims, **characterized in that** the fibers (2) are arranged in the polyurethane foam (1) in the horizontal direction and/or vertical direction and/or chaotically.

## Patentansprüche

1. Füllung eines Sitzes, die einen Polyurethanschaum (1) enthält, wobei die Füllung mindestens zwei Belastungsbereiche (4, 5, 6) aufweist, die einen mit Fasern (2) gesättigten Verbundwerkstoff-Polyurethanschaum (1) enthalten, die fest mit dem Polyurethanschaum (1) verbunden sind, wobei die einzelnen Belastungsbereiche (4, 5, 6) sich in der Dichte der Fasern (2) im Polyurethanschaum (1) unterscheiden, wobei die Belastungsbereiche (4, 5, 6) derart übereinander angeordnet sind, dass der Belastungsbereich mit einer geringeren Dichte der Fasern (2) im Polyurethanschaum (1) über dem Belastungsbereich mit einer höheren Dichte der Fasern (2) im Polyurethanschaum (1) gelagert ist, und wobei im oberen Teil der Füllung sich ein durch den Polyurethanschaum (1) gebildeter Komfortbereich (3) befindet, der keine Fasern (2) aufweist.

2. Füllung nach dem Anspruch 1, **dadurch gekennzeichnet, dass** sie vier Bereiche (3, 4, 5, 6) aufweist, wo im ersten Komfortbereich (3) eine Null-Dichte der Fasern (2) vorliegt, im zweiten Bereich (4) für leichte Belastung die Dichte der Fasern im Polyurethanschaum (1) im Bereich von 1 bis 10 kg/m³ liegt, im dritten Bereich (5) für mittlere Belastung die Dichte der Fasern (2) im Polyurethanschaum (1) im Bereich von 10 bis 15 kg/m³ liegt und im vierten Bereich (6) für hohe Belastung die Dichte der Fasern (2) im Polyurethanschaum (1) im Bereich von 15 bis 20 kg/m³ liegt.

3. Füllung eines Sitzes nach einem der vorangehenden Ansprüche, **dadurch gekennzeichnet, dass** die Fasern (2) im Polyurethanschaum (1) horizontal und/oder vertikal und/oder chaotisch angeordnet sind.

## Revendications

1. Rembourrage de siège contenant de la mousse de polyuréthane (1), où le rembourrage comprend au moins deux zones (4, 5, 6) de charge qui contiennent de la mousse de polyuréthane composite (1) saturée de fibres (2) fixées à la mousse de polyuréthane (1), les différentes zones (4, 5, 6) de charge se distinguant par la densité des fibres (2) dans la mousse de polyuréthane (1), les zones (4, 5, 6) de charge étant disposées les unes au-dessus des autres de telle sorte que la zone de charge présentant la plus faible densité de fibres (2) dans la mousse de polyuréthane (1) est disposés au-dessus de la zone de charge avec une densité plus élevée de fibres (2) dans la mousse de polyuréthane (1), et dans la partie supérieure du rembourrage, la zone de confort (3) est formée par une mousse de polyuréthane (1) qui ne contient aucune fibre (2).

2. Rembourrage selon la revendication 1, **caractérisé en ce qu'il** comprend quatre zones (3, 4, 5, 6) ; dans la première zone de confort (3), la densité des fibres (2) est nulle, dans la deuxième zone (4) de charge légère, la densité des fibres dans la mousse de polyuréthane (1) est comprise entre 1 et 10 kg/m³, dans la troisième zone (5) de charge moyenne, la densité des fibres (2) dans la mousse de polyuréthane (1) est comprise entre 10 et 15 kg/m³ et dans la quatrième zone (6) de charge élevée, la densité des fibres (2) dans la mousse de polyuréthane (1) est comprise entre 15 et 20 kg/m³.

3. Rembourrage de siège selon l'une des revendications précédentes, **caractérisé en ce que** les fibres (2) sont disposées dans la mousse de polyuréthane (1) dans le sens horizontal et/ou dans le sens vertical et/ou de manière aléatoire.
